

G. H. MARSHALL.

PROCESS FOR REDUCING FIBER YIELDING MATERIALS.

APPLICATION FILED JUNE 10, 1909.

971,457.

Patented Sept. 27, 1910.



Witnesses

James F. Brown  
E. M. Ricketts

George H. Marshall <sup>Inventor</sup>  
Watson S. Coleman  
<sup>35</sup> Attorney

# UNITED STATES PATENT OFFICE.

GEORGE H. MARSHALL, OF ROANOKE RAPIDS, NORTH CAROLINA.

## PROCESS FOR REDUCING FIBER-YIELDING MATERIALS.

971,457.

Specification of Letters Patent. Patented Sept. 27, 1910.

Application filed June 10, 1909. Serial No. 501,380.

*To all whom it may concern:*

Be it known that I, GEORGE H. MARSHALL, a citizen of the United States, residing at Roanoke Rapids, in the county of Halifax 5 and State of North Carolina, have invented certain new and useful Improvements in Processes for Reducing Fiber-Yielding Materials, of which the following is a specification, reference being had to the accompanying drawings.

This invention relates to the treatment of fiber yielding materials of the cellulose variety, such as sugar cane, bagasse, cornstalks, sorghum, flax straw, etc. Large quantities 15 of these materials are to be obtained as refuse matter in regions remote from centers where manufacturers might use them for various purposes, such as the manufacture of paper pulp and paper, as well as for textile uses. 20 Owing to the remoteness of the origin of such materials, the matter of transportation makes their cost in many cases prohibitive for the manufacturer. These materials containing cellulose fibers are in many cases destroyed by fire or other methods, and are a 25 source of expense and trouble to the producers, the plants being usually grown for other purposes, such for instance, as sugar cane which is grown for its sugar and flax 30 which is grown for its seed, so that the stalks, as refuse matter, are a total loss to the farmer. It is obvious that it is nearly always impracticable to manufacture these 35 waste materials into commercial products at their points of origin owing to their remoteness from markets and the difficulty of securing skilled labor to utilize such waste materials. It will be quite apparent that if the 40 useless contents of such materials can be moved by a simple cheap process, and the waste materials reduced in weight, say fifty per cent., that it will be possible to make a large saving in freights and thereby place 45 these materials at the disposal of many possible users, both producer and consumer being thus materially benefited and an economy in nature's products promoted. This will be particularly true in the paper and pulp industries, as at the present moment the greatest 50 source of raw materials in these industries is wood of various kinds, the obtention

of which is leading to the rapid depletion of the forests.

It is the object of this invention to provide a simple and cheap process for such 55 utilization of these products, which process consists in treating such waste or raw materials to a high steam pressure in a closed vessel preferably of a rotating type, in the presence of a minimum amount of water and 60 some neutralizing material of an alkaline nature, whereby the sugars, gums and useless incrusting matters are disintegrated and dissolved and rendered possible of removal by blowing the liquor from the closed vessel 65 and afterward subjecting the treated material to washing and drying.

My improved process may be carried out by machinery of various forms and in order that the process may be readily carried 70 out by those skilled in the art, I have illustrated a preferred form in the accompanying drawing in which—

Figure 1 is a diagrammatic illustration, with some of the parts shown in section and 75 some broken away, and Fig. 2 is an elevation of the rotary boiler looking at the right hand thereof as shown in Fig. 1.

Referring specifically to the drawing, 1 indicates a closed vessel or boiler of a well 80 known elongated rotary type, 2, 2, the trunnions upon which the boiler is mounted to rotate, and 3, 4, 5, 6 the gearing which transmits the necessary power for the rotation of the boiler.

The boiler is provided at one end with a discharge spout 7 in which is located a valve 8 of any suitable form to permit of the blowing out of its liquid contents, a swing pipe 9 being connected with the end of the spout, 90 through which the liquid contents, together with the steam used for blowing, and any accumulated gases, may be passed and conveyed to any desired point.

Connected with one of the trunnions 2, 95 which is itself hollow, is a steam inlet pipe 10, the entrance of steam into the boiler being controlled by a suitable valve 11 in said pipe.

The boiler is provided at the end opposite 100 the discharge spout 7 with a suitable cover 12, which may be hinged for convenience of

operation, which cover is rendered hermetically tight by being screwed down by bolts 13 upon a suitable gasket 14. Within the boiler 1, near the discharge end, is a transverse screen 15.

Above and slightly to one side of the boiler is a suitable tank 16 in which the solution to be used in the boiler is mixed, and leading from the bottom of said tank is a 10 pipe 17 having a suitable valve 18, a swing pipe 19 being attached to the end of said pipe 17 in such position that when the pipe 19 is swung down, as shown in dotted lines, the contents of the tank 16 may be discharged into the boiler. Also above and to one side of the boiler is a conveyer of any 15 preferred form, being here shown as an endless belt 20 mounted on pulleys 21, the said conveyer leading to the boiler in order to 20 convey the materials to be treated thereto.

Below the boiler is located a suitable conveyer, here shown as an endless belt 22, on pulleys 23, which serves to convey solid contents discharged from the boiler as hereinafter described, to squeeze rolls 24, and above said rolls, is a water pipe 25 suitably perforated, to discharge water on the matter entering between the rolls. Below the rolls 24 is another conveyer, shown as an endless 30 belt 26 on pulleys 27, which lead to another set of squeeze rolls 28, below which is another conveyer belt 28 mounted on suitable pulleys, as at 30 and leading into a dry house or kiln 31, one of the pulleys supporting belt 29 being within the dry house, which may be heated in any suitable manner, and suitable idler rollers 32 being provided to support the conveyer belt 29 owing to its length.

40 The raw materials are brought to the rotating boiler by the conveyer 20, and discharged into the boiler, the boiler being in a vertical position, with the lid 12 at the top and open.

45 The neutralizing solution being mixed in the tank 16, the swing pipe 19 is lowered into the opening of the boiler and the contents of the tank allowed to flow into the boiler.

50 The neutralizing solution is composed of water with which may be mixed chalk, powdered limestone, lime, or any material of a weak alkaline nature.

A minimum amount of water should be 55 added to the material under treatment in the boiler, and to this end, if the materials are wet, the amount should be approximately a weight of water equal to the weight of the material, and if the material under 60 treatment is quite dry, then there should be a weight of water twice to three times the weight of the material in the boiler.

If the material to be treated is green or very wet, very little water need be added,

in fact less than an equal weight of the 65 water as above stated, because to effectively carry out my process a minimum amount of water must be used, and the steam that condenses supplies some water. I have found that the use of a minimum amount of 70 water or solution together with the heat and direct contact of the steam, and also a sufficient amount of neutralizing alkaline substance enables me to effectively remove sugar, gums and glutinous matters without 75 injuring the fiber proper and the lignin or ligneous incrusting matters which I desire to leave partially if not wholly intact. It is in this particular that my process differs with others heretofore used. The use of a 80 minimum amount of water or solution in the material necessitates the expenditure of a minimum amount of fuel which is required to produce the heat which performs the reduction. The use of a minimum 85 amount of solution not only enables my process to be carried out on the basis of extreme economy in respect to the cost of fuel, but it also exposes the material under treatment to a greater effective steam area. 90

The alkaline contents should be from three to ten per cent. of the weight of material under treatment, the variation of the character of the materials under treatment making it necessary to vary the amount 95 of the neutralizing substances.

By the foregoing statement, namely, that the alkaline contained should be from three to ten per cent. of the weight of the material under treatment I mean the weight of 100 the material when wet or saturated with water; and while these are preferably the proportions used a smaller amount of the alkaline neutralizing substance may be used in the treatment of similar materials.

The materials under treatment, and the neutralizing solution, having been placed in the boiler the cover 12 is then put on and securely bolted to make a tight joint. Steam is then slowly admitted to the boiler through 110 pipe 10 and valve 11 and the boiler rotated on the trunnions by the gearing 3 at a speed of preferably one revolution in two minutes. The steam is allowed to flow into the boiler for say about fifteen minutes when it is cut 115 off and the boiler stopped with the valve 8 at the top, being in a vertical position. The valve 8 is now opened sufficiently to allow the heated air to escape when it is again closed tightly, the boiler again set in motion, and the steam again turned on, the pressure being allowed to rise slowly to about 150 pounds, where it is kept for from one to three hours according to the condition of the material under treatment, green material requiring a short time and old and dry material a much longer period.

The loaded boiler having been kept rotat-

ing and under the steam pressure for from one to three hours, the material within it will have all the gums and useless matter softened sufficiently to permit of blowing down the pressure. The boiler therefore at this period, is stopped in a vertical position, with the valve 8 at the lower end and connection is made to the pipe 9. The valve 8 is now opened as quickly as possible and the resultant liquors in the boiler blown out through the screen 15 which prevents the passage of the material into the pipe 9. The blowing down of the pressure in as short a time as safety will permit, accomplishes a double purpose; first, the quick release of pressure tends to explode the piths or woody portions of the materials in the boiler, such as the pith in sugar cane and the woody boon or stalk in flax straw, and allows this disintegrated matter to pass out more or less with the quick rush of steam through the blow out valve 8. The resultant liquors having been blown out, and the steam pressure having been reduced to atmospheric pressure, the cover 12 is then removed and the boiler turned so that the contents will fall upon the conveyer 22 and be conducted to the squeeze rolls 24, where it receives a shower of water from pipe 25 which washes out the dirt and waste products which failed to pass off in the blow off operation. From the rolls 24 the material passes to another conveyer 26 and thence to a second set of squeeze rolls 28 which remove the surplus water and the material thence passes on the conveyer 29 through the dry house or kiln 31 which may be of any desired or suitable type.

If preferred, the finished product may be dried in the open air and then baled for shipment.

By the foregoing process I do not claim to make a complete or pure finished cellulose product, but I make an average reduction in the weight of the materials of fully fifty per cent., which enables the farmer to profitably ship such partially reduced product to the manufacturer, such partially reduced material, or "half pulp" being capable of being further profitably reduced in manufacturing plants suitably equipped for handling such materials.

It will be noted that my process is only a partial reduction process and must be carried out on the basis of extreme economy in order to be practical. It is therefore important that a minimum amount of water or solution be used so that the cost of fuel will be reduced to a minimum and a minimum amount of neutralizing substance will be necessary. If a large amount of solution is used as in other processes now used, the cost of fuel would exceed the cost of raw material under treatment. Furthermore, when large

quantities of solutions and chemicals are used in carrying out the old process very drastic treatment ensues and the result is the injury to or total separation of the fiber and its ligneous incrusting matter.

Having thus fully described my invention, what I claim as new and desire to secure by Letters Patent, is—

1. The herein described process of treating fiber yielding materials which consists in introducing the materials in a digester together with an alkaline neutralizing agent and a minimum amount of water or moisture, which amount is sufficient to thoroughly saturate the materials and agent, then subjecting the contents of the digester to a mild steam pressure while rotating the digester, then exhausting air and gases from the digester, then gradually increasing the steam pressure within the digester while the materials are being rotated, then suddenly reducing the pressure in the digester and blowing off the materials from the latter, then removing the fibrous materials from the digester and removing the moisture from such materials.

2. The herein described process of treating fiber yielding materials which consists in introducing the materials in a digester, together with an alkaline solution, then subjecting the materials to a mild steam pressure while rotating them, then exhausting the air and gases from the digester, then gradually increasing the steam pressure within the digester while the materials are being rotated, then suddenly reducing the pressure and blowing off the liquids from the digester, then removing the fibrous materials from the digester, and then successively washing the fibrous materials and squeezing the moisture therefrom.

3. The herein described process of treating fiber yielding materials which consists in introducing the materials in a digester, together with an alkaline solution, then subjecting the materials to a mild steam pressure while rotating them, then exhausting the air and gases from the digester, then gradually increasing the steam pressure within the digester while the materials are being rotated, then suddenly reducing the pressure and blowing off the liquids from the digester, then removing the fibrous materials from the digester, then spraying the fibrous materials with water and squeezing them to remove the moisture, then subjecting the fibrous materials to a second squeezing action, and then drying the fibrous materials.

4. The herein described process of treating fiber yielding materials, which consists in introducing the materials in a digester, together with an alkaline solution, then subjecting the materials to a mild steam

pressure while rotating them, then exhausting the air and gases from the digester, then gradually increasing the steam pressure within the digester while the materials are 5 being rotated, then suddenly reducing the pressure and blowing off the liquids from the digester, then removing the fibrous materials from the digester, then spraying the fibrous materials with water and squeezing 10 them to remove the moisture, then subject-

ing the fibrous materials to a second squeezing action, then drying the fibrous material and finally packing the latter for shipment.

In testimony whereof I hereunto affix my signature in the presence of two witnesses. 15

GEO. H. MARSHALL.

Witnesses:

P. H. MURPHY,  
J. T. CHASE.